

No. 674,394.

A. E. BECK & G. TOWNSEND.

Patented May 21, 1901.

TUBE.

(Application filed Nov. 2, 1900.)

(No Model.)



WITNESSES:  
Ella L. Gile  
Otto Munk

INVENTORS.  
Arthur Edward Beck  
George Townsend.

Richard D.

ATTORNEYS

# UNITED STATES PATENT OFFICE.

ARTHUR EDWARD BECK AND GEORGE TOWNSEND, OF BIRMINGHAM, ENGLAND, ASSIGNORS TO PERRINS, LIMITED, OF WARRINGTON, ENGLAND.

## TUBE.

SPECIFICATION forming part of Letters Patent No. 674,394, dated May 21, 1901.

Application filed November 2, 1900. Serial No. 35,217. (No model.)

*To all whom it may concern:*

Be it known that we, ARTHUR EDWARD BECK and GEORGE TOWNSEND, subjects of the Queen of Great Britain and Ireland, and residents of 33 Newhall street, in the city of Birmingham, England, have invented certain new and useful Improvements Relating to Boiler and other Metal Tubes, (for which we have filed an application for a patent in Great Britain, No. 11,981, bearing date July 3, 1900,) of which the following is a specification.

This invention consists of improvements relating to boiler and other metal tubes, our object being to readily and economically produce such tubes from an effective combination of steel and copper or other metals, so that while having ample strength to withstand the stresses imposed upon them they will be better able to resist corrosion than the ordinary tubes at present in use.

On the accompanying sheet of drawings explanatory of our invention, to be hereinafter referred to, Figure 1 is a sectional elevation showing a short thick iron or steel tube or shell in readiness for passing through the rolls, with the mandrel upon which it is to be reduced in thickness and correspondingly lengthened by the rolls and a copper lining for the tube fitting loosely upon the said mandrel. Fig. 2 represents the same parts as Fig. 1, but with the tube in the act of passing through the rolls. Fig. 3 is a sectional view of the finished tube having the copper lining fused thereto.

The same reference-letters are employed in the three views to indicate the same parts.

In the application of our invention to the manufacture of tubes for a water-tube or tubulous boiler in which the water passes through the tubes we place over the mandrel, as A, upon which the hot steel or iron tube shell or comparatively short and thick tube, as B, is to be reduced in thickness and correspondingly lengthened, a cold thin shell or loose sheathing of copper, as C, preferably of a length equal to that of the steel or iron shell B. We then stretch or elongate to

gether both the iron or the steel shell and the copper shell, preferably by subjecting them (while supported by the mandrel A) to the action of rolls D and E in the manner illustrated at Fig. 2. As the parts pass between the rolls the two metals (namely, the iron or steel forming the tube-shell B and the copper C) are pressed into close contact, and as the heat of B is sufficient to fuse the surface of C in contact with it the two metals become very effectually united.

By our process of combining and fusing the copper with the main tube during the ordinary course of its manufacture we are readily enabled to produce at small cost compound tubes with the desired thickness of the respective metals to suit the particular services for which they are required.

We apply our invention to the manufacture of tubes having a copper or other non-corrodible interior, a wrought-iron exterior, and with steel interposed between the two, nesting the three hollow tube blooms or shells the one within the other in the order indicated. We may also make iron or steel tubes or iron and steel tubes with a copper or like exterior and tubes having a copper surface both inside and outside.

Having thus described our invention, what we claim as new, and desire to secure by Letters Patent, is—

The process whereby in the course of the manufacture of boiler and other tubes a covering of non-corrodible metal is fused to the said tubes, consisting in the nesting of a thick and hot tube-shell with a thin and cold sheathing of non-corrodible and more fusible metal, and in subsequently subjecting them together to a compressing, reducing, and elongating action while supported internally by a mandrel, substantially as described.

In witness whereof we have hereunto set our hands in presence of two witnesses.

ARTHUR EDWARD BECK.  
GEORGE TOWNSEND.

Witnesses:

HERBERT BOWKETT,  
HARRY DAVIS.